

June 24, 1930.

C. E. GITHLER

1,767,923

METHOD OF MAKING TUBING

Filed May 31, 1928

2 Sheets-Sheet 1

*Fig. 1.*



*Fig. 2.*



*Fig. 3.*



*Fig. 4.*



*Fig. 5.*



*Fig. 6.*



*Fig. 7.*



*Fig. 8.*



INVENTOR

Charles E. Githler.

BY 

ATTORNEYS.

June 24, 1930.

C. E. GITHLER

1,767,923

METHOD OF MAKING TUBING

Filed May 31, 1928

2 Sheets-Sheet 2



INVENTOR  
Charles E. Githler.  
BY  
Doway  
ATTORNEYS.

# UNITED STATES PATENT OFFICE

CHARLES E. GITHLER, OF CORNING, NEW YORK, ASSIGNOR TO CORNING GLASS WORKS,  
OF CORNING, NEW YORK, A CORPORATION OF NEW YORK

## METHOD OF MAKING TUBING

Application filed May 31, 1928. Serial No. 281,779.

This invention relates to the art of tubing and more particularly to a process of manufacturing tubing having a stripe of contrasting color in proximity to the bore.

5 In previous methods of making such tubing considerable difficulties have been experienced in controlling the width and position of the stripe, and it is an object of the present invention to provide an improved 10 method of making striped tubing.

With the above and other objects in view, which will be apparent as the description proceeds, I have set forth my invention in the following specification and illustrated 15 it in the accompanying drawings, in which:

Figs. 1-10 are longitudinal sections through the end of a blow pipe and a gather of glass thereon showing successive steps in the manufacture of striped tubing by my 20 new method, Fig. 10 being shown on a considerably reduced scale;

Figs. 11 and 12 are longitudinal and transverse sections showing the next step in my method of making tubing;

25 Figs. 13 and 14 are similar views of a further step in my method;

Figs. 15 and 16 are similar views showing a still further step in my method;

Fig. 17 is a transverse section corresponding to Fig. 16 but showing a modified form 30 of tubing; and

Figs. 18 and 19 are a transverse section and a partial vertical elevation, respectively, 35 on an enlarged scale, of finished tubing made from a blank having the cross section shown in Fig. 17.

According to the preferred form of my method a quantity of clear glass 21 is gathered on the end of a blow iron 22 (Fig. 1). 40 This is then marvered, preferably with the aid of a flat paddle (not shown), until it is given a circular cross section (Fig. 2).

The glass is then indented at 23 in the vicinity of the end of the blow iron and at 45 24 near the tip of the gather (Fig. 3), the

indenting at 23 serving to prevent the glass 25 which is in direct contact with the sides of the blow iron from pulling away therefrom in the further operations to which it is subjected, and the indenting at 24 serving to confine the extent of the blow (described later) and to provide a convenient hold for the subsequent elongation of the gather. The operator then blows through the blow iron 22 to form a cavity 25' (Fig. 4) that eventually forms the bore of the tubing. The operator then seizes the portion 26 which extends beyond the indentation 24 and pulls it outwardly to slightly elongate the cavity, and he further indents the 50 gather at 27, which is at a point overlapping the cavity. The extending portion 26 is then cracked off by means of an ordinary glass worker's tool (not shown), leaving the end 28 of the cavity exposed (Fig. 55). The operator then flares the gather 60 outwardly (Fig. 7) and inserts a stripe of colored glass 29 in the flared gather with the far end of the colored glass extending 65 slightly into the bore of the blow iron (Fig. 6). The operator then flares the gather 70 outwardly (Fig. 7) and inserts a stripe of colored glass 29 in the flared gather with the far end of the colored glass extending slightly into the bore of the blow iron (Fig. 7). The operator then closes the cavity 75 and indents it at 30 to provide a convenient hold for the next operation, which is to draw the gather outwardly, after which he indents it at 30' to define the portion of the gather which is to be incorporated in the 80 finished blank. This projecting portion 31 is then cracked off (Fig. 9), thus completing the initial steps in the formation of the tubing blank.

The remaining steps are then the same as those ordinarily used in the manufacture of tubing and consist in gathering additional clear glass around the flint glass 32 to form the gather 33 (Fig. 10), gathering 85 more clear glass and imparting a ball shape to this gather (Figs. 11 and 12), elongating the gather by marvering and swinging until the bore is of the proper length and shape, and applying a stripe of 90

white enamel 34 on the outside of the gather but on the same side of the bore as the colored stripe 29 (Figs. 13 and 14). Additional glass 35 is then gathered (Figs. 15 and 16) and, if lens front tubing is to be made, the shape shown in Fig. 17 is imparted to the blank by lensing in the regular way.

The blank is then ready for reheating 10 and drawing out into tubing 36 as shown in Figs. 18 and 19. As indicated in Fig. 19 a column of fluid 37 placed in the bore of the tubing will be magnified so as to substantially fill the tube up to the height 15 of the liquid, and above this there will be exposed, as a direct continuation of this fluid, the colored stripe 29 which was incorporated into the gather. On either side of both the fluid and the colored stripe and extending 20 throughout the height of the tubing is the light shield 34, if the tubing is provided with a light shield, and upon both sides of the light shield will be visible the flint glass 35.

25 The glass is reheated from time to time, in the ordinary way, during the carrying out of the above operations.

It will be understood that the final shape 30 of the tubing may be round as shown in Fig. 16, lensed as shown in Fig. 17, or any other shape which it is desired to impart to the blank, that the bore may be made round, oval or any other desired shape, that the body and stripe may be made of any desired 35 combination of glasses, and that the light shield may be used or not as desired.

It will therefore be apparent that I have developed a new and useful method of making tubing which permits the correct positioning 40 of the colored stripe at the desired position in the blank, and that its size may be readily controlled by the size of the inserted mass of glass (Fig. 7). Furthermore, if desired, a combination of stripes can be 45 inserted in connection with the step shown in Fig. 7 instead of a single stripe.

I claim:

1. The method of making tubing which 50 consists in gathering molten glass on the end of a blow pipe, marvering it, blowing a cavity in the glass, opening the cavity, placing a strip of glass in the cavity, closing the opening, gathering additional glass, elongating, marvering and drawing out the gather 55 to form tubing of the desired size.

2. The method of making tubing which 60 consists in collecting molten glass on the end of a blow pipe, shaping it, forming a cavity, opening up the cavity at one end and inserting colored glass within the bore, closing the cavity, recovering and drawing.

3. The method of making tubing which 65 consists in gathering molten glass on the end of a blow pipe, marvering it, blowing a cavity 70 in the glass, opening the cavity, placing a

strip of glass in the cavity, closing the cavity, gathering additional glass therearound, marvering it, elongating the cavity and forming a bore of the desired shape, gathering additional glass therearound, marvering 75 the gather to give it the desired shape of the finished tubing, and drawing out the gather to form tubing of the desired size.

4. The method of making tubing which 75 consists in gathering molten glass on the end of a blow pipe, marvering it, indenting it in proximity to the end of the blow pipe, blowing a cavity in the glass, removing the outer end of the gather to expose the end of the cavity, placing a strip of glass in the gather, 80 gathering additional glass therearound, marvering it, elongating the cavity and forming a bore of the desired shape, gathering additional glass therearound, marvering 85 the gather to give it the desired shape of the finished tubing, and drawing out the gather to form tubing of the desired size.

5. The method of making tubing which 90 consists in gathering molten glass on the end of a blow pipe, marvering it, indenting it in proximity to the end of the blow pipe, blowing a cavity in the glass, removing the outer end of the gather to expose the end of the cavity, opening said gather, placing a strip of glass in the gather with its far end extending into the end of the bore of the blow pipe, closing the gather, gathering additional glass therearound, marvering it, elongating 95 the cavity and forming a bore of the desired shape, gathering additional glass therearound, marvering the gather to give it the desired shape of the finished tubing, and drawing out the gather to form tubing of the desired size.

6. The method of making tubing which 105 consists in gathering molten glass on the end of a blow pipe, marvering it, indenting it in proximity to the end of the blow pipe, blowing a cavity in the glass, pulling the tip of the gather outwardly to constrict the outer 110 end of the cavity, removing said outer end of the gather to expose the end of the cavity, opening said gather, placing a strip of glass in the gather with its far end extending into the end of the bore of the blow pipe, closing the gather, gathering additional glass 115 therearound, marvering it, elongating the cavity and forming a bore of the desired shape, gathering additional glass therearound, marvering the gather to give it the 120 desired shape of the finished tubing, and drawing out the gather to form tubing of the desired size.

7. The method of making tubing which 125 consists in gathering molten glass on the end of a blow pipe, marvering it, indenting it in proximity to the end of the blow pipe, blowing a cavity in the glass, pulling the tip of the gather outwardly to constrict the outer end of the cavity, removing said outer 130

end of the gather to expose the end of the cavity, opening said gather, placing a strip of glass in the gather with its far end extending into the end of the bore of the blow pipe, closing the gather, removing the outer end of the gather without exposing the cavity, gathering additional glass therearound, marvering it, elongating the cavity and forming a bore of the desired shape, applying a light shield to the gather on the same side of the bore as the inserted glass, gathering additional glass therearound, marvering the gather to give it the desired shape of the finished tubing, and drawing out the gather to form tubing of the desired size.

CHARLES E. GITHLER.

20

25

30

35

40

45

50

55

60

65